

## 1

2,940,811

METHOD FOR IMPARTING COLOR TO  
CEDARWOOD

Edward Farber, Washington, D.C., assignor, by mesne assignments, to Great Western Producers, Inc., Gulf Red Cedar Company Division, New York, N.Y., a corporation of Maryland

No Drawing. Filed Oct. 6, 1959, Ser. No. 844,622

16 Claims. (Cl. 8—6.5)

This invention relates to the preparation of cedarwood for the manufacture of pencils. More particularly, the invention relates to a novel process effective to impart a reddish color to the heart and sapwood of incense cedar.

It is conventional practice in the prior art to treat cedarwood from which pencils are manufactured to impart thereto a generally uniform reddish color by impregnation of cedar slats with a solution of an appropriate dye, normally an azo-dyestuff. More specifically, in accordance with such prior art processes, cedar slats are moved through pressure vessels containing a dyestuff solution. Vacuum and superatmospheric pressure conditions are required to effect saturation by impregnation of the cedarwood slats with the dyestuff solution. During the period of residence in the pressure vessels, normally at least about a few hours, the cedarwood slats increase in weight about 150% to 200% by reason primarily of water absorption. Water so absorbed must be removed over a long period of time in a carefully regulated, drying operation which normally requires from about ten to about fourteen days, and necessitates the maintenance of a large inventory of pencil slats in process.

It is accordingly a primary object of this invention to provide an improved method for imparting a satisfactory red coloration to cedarwood pencil slats.

It is a more specific object of the invention to provide a method for the production of a satisfactory red color in cedarwood slats which does not require the utilization of vacuum or superatmospheric pressure conditions.

It is an additional object of the invention to provide a process for imparting a satisfactory color to cedar pencil slats pursuant to which treated slats can be effectively dried without material adverse effect a substantially shorter time period than is required by prior art methods.

It is yet a further object of the invention to provide an economical method for imparting a satisfactory red color to cedarwood pencil slats which can be completed in a materially shorter period of time than conventional processes for achieving a like result.

A more specific object of the present invention to provide a process pursuant to which an alkali metal nitrite and a dyestuff are used in conjunction to impart a color to cedarwood appropriate for use in pencil manufacture.

It is an additional object of the invention to provide an effective two-stage process for imparting an appropriate reddish coloration to cedarwood pencil slats pursuant to which a dyestuff is so employed as to obviate the time-consuming impregnation procedures essential to prior art expedients entailing dyestuff utilization.

In accordance with this invention, it has been discovered that a reddish coloration satisfactory for pencil manufacture can be imparted to cedarwood by contacting said cedarwood with an aqueous solution containing from about 1% to about 6% by weight of an alkali metal nitrite under conditions to effect absorption by said wood of from about 0.03% to about 5.0% by weight of said nitrite and thereafter gradually removing water from the nitrite-containing wood over a time period of at least

## 2

about twelve hours to produce a colored cedarwood product containing not more than about 10% water.

In accordance with a more specific aspect of the invention, it has been discovered that a red coloration satisfactory for pencil manufacture can be imparted to cedarwood by a process which comprises first contacting cedarwood with an aqueous solution containing from about 1% to about 6% by weight of an alkali metal nitrite and thereafter contacting said cedarwood with an aqueous solution of a dyestuff of appropriate coloration, said cedarwood absorbing in said process from about 0.03% to about 5.0% by weight of alkali metal nitrite, and thereafter gradually removing water from the nitrite-containing cedarwood over a period of at least about 12 hours to produce a colored cedarwood product containing not more than about 10% by weight of water.

Pursuant to the invention, aqueous solutions of all alkali metal nitrates can be employed, including specifically sodium, potassium and lithium nitrite. Sodium nitrite is preferred. The aqueous alkali metal nitrite solutions utilized normally do not contain more than about 6% by weight of nitrite to foreclose the formation of an undesired dark color in the outer layers of the cedarwood treated. In the practice of the invention to produce a product in which such darker colors are not disadvantageous, alkali metal nitrite concentrations in excess of 6% by weight can be utilized. A practical lower limit of nitrite concentration is about 0.1% by weight. Preferably, alkali metal nitrite solutions containing from about 3% to about 5% by weight of alkali metal nitrite are employed.

The process of the invention is appropriately practiced at atmospheric temperature, normally about 20° C., although any temperatures between the freezing and boiling points of the aqueous treating solution can be employed. A temperature range of from about 60° C. to about 90° C. is preferred.

Atmospheric pressure is preferable in the practice of the invention. Utilization of superatmospheric pressure or subatmospheric pressure or a combination thereof to facilitate impregnation of the slats with the treating solution in conventional manner is not precluded but is not essential to the success of the invention.

Cedarwood undergoing treatment in accordance with the invention is maintained in contact with the treating solution for a period of time requisite to provide a concentration of nitrite in the wood within the range of from about 0.03% to about 5.0% by weight. When treating solutions containing from about 1% to about 6% by weight of alkali metal nitrite are employed, the total quantity of the solution absorbed by the wood will vary from about 30% to about 80%, preferably from about 40% to about 60%, by weight of the wood.

The cedarwood should not remain in contact with the treating solution for more than about one hour to minimize the possibility of adverse effect on the color of the final product. Prolonged treatment, particularly at elevated temperatures, reduces the natural color of the heartwood. It is, accordingly, preferred to complete the treatment within a period of not more than about 60 minutes. Treating periods of about twenty minutes or less are frequently adequate.

To facilitate and expedite the absorption of the treating solution by the wood, it is preferable to vary the treating temperature during the contact period. Accordingly, a preferred embodiment of the invention entails a two-stage treatment including as a first stage a treating period of relatively short duration at higher temperatures in excess of about 50° C., preferably from 60° C. to about 90° C., for a period of about not more than about 60 minutes, preferably from about 15 to about 30 minutes; and, as a second stage in which the

first stage product is contacted with a treating solution substantially cooler, preferably at least about 10° C., than the first stage solution for a period of not more than about 15 minutes, preferably from about 2 to about 10 minutes. The second stage treating solution is employed at a temperature of not more than about 80° C., preferably from about 20° C. to about 40° C.

It will be appreciated that in accordance with the two-stage method of practicing the invention, the concentrations of the treating solutions in the respective stages can appropriately be varied. Normally, a more concentrated solution is employed in the first stage. For example, it is appropriate to use a relatively concentrated solution containing from about 4% to about 6% by weight of an alkali metal nitrite in the first or high temperature stage, and a more dilute solution containing from about 1% to about 3% or 4% by weight of alkali metal nitrite in the second or low temperature stage.

Water is removed from cedarwood treated in accordance with the invention over a period of at least about 12 hours to facilitate uniform distribution of the alkali metal nitrite in the wood while the wood is wet and to preclude accumulation of the nitrite close to the wood surface. Water removal is effected in this manner to produce a colored cedarwood product which contains not more than about 10%, and preferably from about 5% to about 10%, by weight of water. A layer of darkened wood of unsatisfactory color may be produced, particularly when the more concentrated solutions containing 5% or more by weight of alkali metal nitrite are employed.

The production of such disadvantageous darkening is foreclosed by the two-stage process in which the second stage of impregnation is effected at a relatively low temperature with a nitrite solution of lower concentration. Alternatively, such disadvantages darkened layers can be avoided by rinsing the single stage treated cedarwood with water. A relatively fast dip in warm water is adequate.

The precise chemical action by which the alkali metal nitrite produces the desired coloration in the cedarwood is not fully understood. Since only a very small effective quantity of nitrite is utilized, it is considered likely that the nitrite reacts with terpene derivatives in the wood, such as libocedrol, in their natural environment to produce the desired color.

In that embodiment of the process of the invention in which a dyestuff is employed after nitrite treatment, atmospheric temperatures and pressures are also approximately utilized, although all temperatures within the range between the freezing point of the dyestuff solution and the boiling point thereof can be employed. Subatmospheric or superatmospheric pressure conditions or combinations thereof are not essential but can be employed in conventional manner to facilitate the absorption of the dyestuff by the wood.

In accordance with the modification of the invention, in which a two-step alkali metal nitrite impregnation process is used in the first stage, the dyestuff can be added to the alkali metal nitrite solution utilized in the second step. Such a mode of operation is, however, not preferred by reason of the adverse effect of the dyestuff in the absorption in formation of color in the wood.

Any appropriate dyestuff can be utilized, normally in a concentration of from about  $\frac{1}{10}$  of one part by weight to about 70 to 200 parts by weight of the aqueous solution. Representative dyestuffs which may be suitably employed are aniline, quinoline and anthraquinone dyestuffs.

More specifically, Naphthol Yellow S, Ponceau, Methyl Violet, natural dyestuffs including logwood and indigo and the like are contemplated. Appropriate azo dyes are listed at pages 261 to 293, appropriate anthraquinone dyes at pages 343 to 350, appropriate aniline dyes at pages 337 and appropriate quinoline dyes at page 328 of Gilman, "Organic Chemistry, an Advanced Treatise." Reference

is made to "The Chemical Formulary," vol. IV, page 346 (1939), and vol. V, page 284, Chemical Publishing Co., Inc., for the disclosure of wood dyeing techniques. Smith Patent 2,713,364 and German Patents 422,124 and 439,226 also describe wood dyeing processes, and dyes useful therein.

#### Example I

A group of approximately 100 dried, incense cedar, about  $2\frac{1}{8}'' \times 3\frac{1}{8}'' \times 7\frac{1}{4}''$  pencil slats weighing about 515 lbs. was immersed in a water solution containing about 2% by weight of sodium nitrite and maintained at a temperature of about 85° C. for a period of about fifteen minutes. At the termination of the first fifteen minute period, the treating solution containing the slats was cooled during an additional fifteen minute period to about 60° C. The slats were maintained immersed in the 60° C. solution for a third fifteen minute period and then removed. The heated slats reflected a weight increase of about 47% of the original weight thereof by reason of the absorption of the treating solution. The treated slats were then maintained in a confined space with minimum air circulation for a period of about eight hours and thereafter exposed to drying conditions in a stream of warm air characterized by a temperature within the range of about 50° C. to about 75° C. After about five days under such drying conditions, it was found that the moisture content of the treated slats is reduced to from about 5% to about 10% by weight, and that a satisfactory red color for the production of pencils had developed in the slats.

By way of comparison, similar slats treated identically, with the exception that the treated slats were dried rapidly over a period of only about six hours to a moisture content of from about 5% to about 10% by weight, developed only slight coloration and were unsatisfactory for the manufacture of pencils.

#### Example II

40 Cedarwood slats of the same type and in the same amount as described in Example I were immersed in a 5% by weight water solution of sodium nitrite at a temperature of 90° C. for a period of ten minutes, removed from the 5% treating solution, and thereafter immersed 45 in a like solution containing only about 1% by weight of sodium nitrite at a temperature of about 40° C. The slats so processed were dried slowly in the same manner as described in Example I. A uniform red color satisfactory for the manufacture of pencils developed in the 50 treated slats.

#### Example III

A quantity of slats equal in weight and description to those described in Example I were immersed in a water solution containing 4% by weight of sodium nitrite and 55 2% by weight of urea maintained at a temperature of 70° C. After ten minutes of such immersion, the slats increased in weight by 26% and were thereafter immersed in a solution containing 2% sodium nitrite and 1% urea at a temperature of 30° C. for a period of about fifteen 60 minutes. The slats removed from the second treating solution were found to weight 48% more than the original untreated slats. After slow drying in the manner described in Example I, the treated slats were found to be 65 uniformly colored red in a manner satisfactory for the production of pencils.

#### Example IV

A group of cedar slats identical with those described in 70 Example I are immersed in the first stage in a water solution containing 4% by weight of sodium nitrite and 3% by weight of urea maintained at a temperature of 75° C. for a period of thirty minutes. The slats were then removed from the first stage treating solution and immersed 75 in a water solution containing 2% by weight of paraffin in

5 emulsion maintained at a temperature of 30° C. for fifteen minutes.

After removal from the second treating solution and drying in the manner described in Example I, the cedar slats were found to be appropriately colored red and suitable for use in the manufacture of pencils.

It will be appreciated that softening agents other than urea and paraffin emulsions such as polyethylene glycols, invert sugar, and the like, can be employed in conjunction with the alkali metal nitrite treating solutions of the invention to produce a desirable degree of softness in the treated cedarwood product. For example, water solutions containing from about 2 to about 5 parts, preferably about 4 parts, by weight of alkali metal nitrite and from about 1 to about 3 parts, preferably about 2 parts, by weight of polyethylene glycol having an average molecular weight of about 200 can be employed. Similarly, a water solution containing from about 2 to about 5 parts, preferably about 4 parts, by weight of alkali metal nitrite and about 3 to about 6 parts, preferably about 4 parts, by weight of invert sugar can be employed. In general, the range of concentrations of such softening agents in the treating solutions of the invention is from about 2% to about 5% by weight.

A further specific embodiment of the invention contemplates the utilization of resorcinol in conjunction with an alkali metal nitrite in the production of a satisfactory reddish coloration in cedarwood pencil slats. In accordance with such embodiment of the invention, resorcinol is employed in the aqueous alkali metal nitrite treating solutions, preferably in proportions of from about 0.1% to about 3% by weight. The resorcinol is employed either in the one-stage or in the two-stage mode of practicing the invention. When utilized in the two-stage method, the resorcinol is appropriately employed solely in the first stage, solely in the second stage, or jointly in both stages.

The following example is illustrative of the practice of the invention utilizing resorcinol.

#### Example V

Cedarwood slats, of the same type and in the same number as described in Example I, are immersed for about 40 minutes in a water solution containing about 1% by weight of sodium nitrite and about 1.6% by weight of resorcinol, maintained at a temperature of about 80° C. The solution containing the cedarwood slats is then cooled to about 50° C. and the slats are maintained immersed in the 50° C. solution for about 15 additional minutes. The slats, upon removal from the treating solution, are found to have absorbed about 70% by weight thereof and are satisfactorily colored after drying in the manner described in Example I.

#### Example VI

A group of 100 incense cedar slats containing about 7% moisture, about 2 1/2" x 3/8" x 1 1/4" in dimension, and weighing 2652 grams were immediately immersed in a 5% water solution sodium nitrite maintained at 70° C. for about 30 minutes. The treated slats upon removal from the treating solution weighed 3476 grams and were immediately immersed in a water solution of 0.07% by weight of a commercial azo-dyestuff maintained at a temperature of about 40° C. for a period of about five minutes. The dyestuff employed was a sulfonate. The weight of the slats upon removal after five minutes immersion in the dyestuff solution was 3953 grams. The treated slats were then dried by subjection to a temperature of about 75° C. for twelve hours in a humid atmosphere during which time only slight evaporation of water took place, followed by exposure to drying took place, followed by exposure to drying conditions in a stream of warm air characterized by a temperature within the range of about 50° C. to about 75° C. for a period of about 2 days to produce a final, dried, colored

6 product containing about 7% by weight of water and appropriately colored both internally and externally for the manufacture of pencils.

#### Example VII

A group of slats, similar to that described in reference to Example VI, was immersed in a water solution containing 4% by weight of sodium nitrite for ten minutes at 90° C. at atmospheric pressure. The slats were then 10 removed from the sodium nitrite treating solution and immersed in a solution containing 1% by weight of sodium nitrite and 0.1% by weight of the same azo-dyestuff described in Example VI. The slats were removed from the second treating solution after about ten minutes 15 at a temperature of about 50° C. The treated slats reflected a weight increase of about 55%. The slats so produced were dried in the same manner as the slats in Example VI to produce a similar product.

#### Example VIII

A group of slats of incense cedar, of the same type described in Example VI were immersed in atmospheric pressure in a 4% solution of sodium nitrite maintained at a temperature of about 90° C. After immersion 20 25 for ten minutes, the treating solution was cooled to about 80° C. and the slats were removed therefrom. It was determined that the slats had increased in weight by 36% by reason of absorption of the treating solution.

By way of comparison, an identical process was 30 repeated with the exception that the treating solution contained, in addition to 4% by weight of sodium nitrite, 0.1% by weight of the brown azo-dyestuff described in reference to Example VI. The cedar slats subsequent to the treatment reflected an increase in weight of only 35 about 20.5%, thus reflecting the adverse effect of the dyestuff on the absorption of the nitrite treating solution by the cedarwood. Moreover, the slats produced in accordance with the process first described, after slow drying in the manner described in reference of Example VI, 40 demonstrates excellent internal coloration, whereas the slats resulting from the second treatment, in which the dyestuff is employed, demonstrated very little coloration of the wood, although the surface of the slats was adequately colored.

#### Example IX

Example VII is repeated with the exception that the dyestuff solution employed in the second stage contained 2.5% by weight paraffin in emulsified form. The dried 50 product produced was characterized by an enhanced softness appropriate for pencil manufacture. The quantity of dyestuff absorbed on the cedarwood surface corresponded to about 0.03% by weight of the cedarwood. In prior art procedures entailing the utilization of vacuum and pressure for effecting the coloring of cedarwood slats of dyestuffs, at least about 0.2% by weight of dyestuff is consumed.

It will be appreciated that other softening agents and 55 paraffin emulsions, such as polyethylene glycols, invert sugars, and the like, can be employed in either stage of the process of the invention to produce a desirable degree of softness in the colored cedarwood product. For example, treating solutions containing from about 2 to about 5, preferably about 4, parts by weight of alkali metal nitrite, and from about 1 to about 3, preferably about 2 parts, by weight of polyethylene glycol having an average molecular weight of about 200 can be employed in the first stage. A like amount of polyethylene glycol can be employed in the second stage. Similarly, 60 a water solution containing from about 2 to about 5, preferably about 4, parts by weight of alkali metal nitrite and about 3 to about 6, preferably about 4, parts by weight of invert sugar can be employed in the first stage. Corresponding amounts of invert sugar can be employed 65 in the second stage. In general, the range of concentra-

tion of softening agents in the treating solutions in either stage of the process of the invention fall within the range of from about 2% to about 5% by weight.

This application is a continuation-in-part of Farber application Serial No. 651,582 and Farber application Serial No. 651,583, both filed April 9, 1957, and both now abandoned.

I claim:

1. The process for imparting a reddish coloration satisfactory for pencil manufacture to cedarwood slats which comprises, contacting said cedarwood with an aqueous solution containing from about 1% to about 6% by weight of an alkali metal nitrite under conditions to effect absorption by said wood of from about 0.03% to about 5.0% by weight of said nitrite and thereafter gradually removing water from the nitrite-containing wood over a time period of at least about 12 hours to produce a colored cedarwood product containing not more than about 10% water.

2. The process of claim 1 wherein the alkali metal nitrite is sodium nitrite.

3. The process of claim 1 carried out at a temperature of from about 60° C. to about 90° C.

4. The process of claim 1 wherein said alkali metal nitrite solution contains from about 3% to about 5% by weight of alkali metal nitrite.

5. The process of claim 1 wherein said alkali metal nitrite treating solution contains a softening agent selected from the group consisting of urea, aqueous emulsions of paraffin wax finely dispersed through emulsifying agents, polyethylene glycols, and invert sugar.

6. The process of claim 1 wherein said aqueous solution of an alkali metal nitrite contains from about 0.1% to about 3% by weight of resorcinol.

7. The process for imparting a reddish coloration satisfactory for pencil manufacture to cedarwood which comprises a first stage in which the cedarwood is contacted with an aqueous solution of an alkali metal nitrite containing from about 4% to about 6% by weight of alkali metal nitrite at a temperature in excess of about 50° C. for a period of not more than about 60 minutes, and a second stage in which the first stage product is contacted with an aqueous solution of an alkali metal nitrite at least about 10° C. cooler than the first stage treating solution and containing from about 1% to about 3% by weight of alkali metal nitrite for a period of not more than about 30 minutes.

8. The process of claim 7 wherein said second stage treating solution is employed at a temperature of from about 20° C. to about 40° C.

9. The process of claim 7 wherein at least one of said first stage and second stage treating solutions contain

from about 0.1% to about 3% by weight of resorcinol.

10. A process for imparting a red coloration satisfactory for pencil manufacture to cedarwood comprising a first stage (a) in which a cedarwood is contacted with an aqueous solution containing from about 1% to about 6% by weight of an alkali metal nitrite, and a second stage (b) in which the first stage product is contacted with an aqueous solution of a dyestuff of appropriate coloration for dyeing cedarwood, said cedarwood absorbing in said process from about 0.03 to about 5.0% by weight of alkali metal nitrite, and thereafter gradually removing water from the nitrite-containing cedarwood over a period of at least about 12 hours to produce a colored cedarwood product containing not more than about 10% by weight of water.

11. The process of claim 10 wherein said first stage (a) and said second stage (b) are practiced at substantially atmospheric pressure.

12. The process of claim 10 wherein said first stage (a) is carried out in two steps, including a first step in which an alkali metal nitrite solution containing from about 4% to about 6% by weight of alkali metal nitrite is employed, and a second step in which from about 1% to about 4% by weight of alkali metal nitrite is employed.

13. The process of claim 12 wherein said first step is practiced at a temperature of from about 60° C. to about 90° C., and wherein said second step is practiced at a temperature at least about ten degrees lower than said first step.

14. The process of claim 10 wherein there is employed in said second stage (b) an aqueous solution of a dyestuff containing, in addition to said dyestuff, from about 1% to about 3% by weight of an alkali metal nitrite.

15. Cedarwood colored in accordance with the method of claim 10.

16. The process of claim 10 wherein said aqueous solution contains a softening agent selected from the group consisting of urea, polyethylene glycols, invert sugars and aqueous emulsions of paraffin wax finely dispersed through emulsifying agents.

#### References Cited in the file of this patent

##### UNITED STATES PATENTS

|           |           |               |
|-----------|-----------|---------------|
| 1,135,167 | Doyen     | Apr. 13, 1915 |
| 2,395,311 | Woodhouse | Feb. 19, 1946 |
| 2,517,296 | Farber    | Aug. 1, 1950  |
| 2,733,119 | Nach      | Jan. 31, 1956 |

##### FOREIGN PATENTS

|         |               |               |
|---------|---------------|---------------|
| 296,547 | Great Britain | Sept. 6, 1928 |
|---------|---------------|---------------|